

# UNITED STATES PATENT OFFICE.

OSCAR MURISIER, OF ALEXANDROWSKY, NEAR ST. PETERSBURG, RUSSIA,  
AND PERCY CARLYLE GILCHRIST, OF PALACE CHAMBERS, WESTMINSTER,  
ENGLAND; SAID MURISIER ASSIGNOR TO SAID GILCHRIST.

## JUNCTION OR SEPARATOR LINING FOR OPEN-HEARTH FURNACES.

SPECIFICATION forming part of Letters Patent No. 329,937, dated November 10, 1885.

Application filed May 4, 1885. Serial No. 164,373. (No specimens.)

*To all whom it may concern:*

Be it known that we, OSCAR MURISIER and PERCY CARLYLE GILCHRIST, respectively a citizen of the Swiss Republic, residing at Alex-  
5 androwsky, near St. Petersburg, Russia, and a subject of the Queen of Great Britain, residing at Palace Chambers, Westminster, Eng-  
land, have invented a certain new and useful  
10 Improvement in Junction or Separator Lin-  
ings for Open-Hearth Furnaces, of which the  
following is a specification.

In the manufacture of steel in the Siemens  
or open-hearth furnace by what is known as  
the "basic" or "Thomas Gilchrist" process,  
15 much difficulty has been experienced when  
the silica roof and sides have been allowed to  
rest directly upon the basic hearth, as in such  
case the silica combines with the basic mate-  
rial and rapidly melts away, bringing down  
20 with it the sides and ports of the furnace.

The object of our invention is to remedy  
this defect, and to this end we employ chrome  
ore made plastic with tar as a separator or  
junction between the basic and silicious mate-  
25 rials, such junction being preferably above  
the slag-level. Such mixture, we find, does not  
flux with either the basic or silica materials,  
and may be readily put in place by ramming  
in the ordinary manner, or may be used in the  
30 form of bricks prepared by mixing the chrome  
ore with just sufficient tar to make the mass  
plastic, such mass being then molded under  
pressure into the form of bricks, which may  
or may not receive a preliminary firing before  
35 being placed in position. The chrome ore  
and tar junction (whether rammed *in situ* or  
used in the form of bricks) need only be of a

few inches in thickness, and will rest directly  
upon the basic material, while the silica will  
rest directly upon it. 4c

We are aware that it has been before pro-  
posed to use chrome ore and oxide of chromium  
for lining furnaces, as in United States Letters  
Patent No. 308,984, such lining being highly  
resistant and interposed between the bath of 4.  
metal and the ganister or other lining, and  
covering the whole of such lining; but such  
materials have not, so far as we know, been  
mixed with tar and used simply as a junction  
or separator, and 5

What we therefore claim, and desire to se-  
cure by Letters Patent, is—

1. A mixture of chrome ore and tar, com-  
pounded substantially as set forth, for use in  
separating or forming the junction between 5  
the basic and acid portions of the linings of  
metallurgical furnaces.

2. A furnace-lining composed of a basic bot-  
tom, basic sides, and acid roof, and a belt of  
a mixture of chrome ore and tar interposed 6  
between the roof and sides, as set forth.

In witness whereof we have hereunto set our  
hands, each in the presence of two subscribing  
witnesses.

OSCAR MURISIER.

PERCY CARLYLE GILCHRIST.

Witnesses to the signature of Oscar Murisier:

AM. ARMAND,

M. DUFOUR.

Witnesses to the signature of Percy Carlyle  
Gilchrist:

JNO. DEAN,

W. J. NORWOOD,

Both of 17 Gracechurch Street, London.